

Jan. 13, 1953

R. J. MOORE

2,625,510

LUBRICATING GREASE COMPOSITION

Filed Oct. 25, 1951



Inventor:

Robert J. Moore  
By James Jodarovic  
His Attorney

## UNITED STATES PATENT OFFICE

2,625,510

## LUBRICATING GREASE COMPOSITION

Robert J. Moore, Oakland, Calif., assignor to Shell Development Company, Emeryville, Calif., a corporation of Delaware

Application October 25, 1951, Serial No. 253,110

20 Claims. (Cl. 252—37)

1

This invention relates to improved lubricating grease compositions. More particularly, it pertains to novel grease compositions which resist bleeding and age-hardening and which possess outstanding mechanical stability and thermal reversibility.

It is well established that oxidation has a profound deteriorating effect upon lubricants and lubricating compositions. The rapidity of this deterioration varies with different lubricants and depends in part upon the source of the base oil, the presence and nature of additives therein, as well as on the conditions to which the lubricant is exposed. Once oxidation has started in a lubricant, the deterioration caused thereby appears to be an autocatalytic phenomenon, resulting in further deterioration of the lubricant.

Bleeding is a phenomenon frequently encountered in grease compositions, this bleeding being manifested by an undesirable separation of the soap and lubricant, comprising the grease mixture, into fluid oil and a portion richer in soap. This action has also been termed syneresis, and it is thought to be due to changes occasioned by some instability in the soap-hydrocarbon structure.

Generally, to inhibit bleeding and to improve the texture of greases, special precautionary measures are taken, such as employing slow or rapid means of cooling, or extensively working the grease in special homogenizers, e. g. the Cornell homogenizer, and the like. Such procedures are usually time consuming and add greatly to the cost of the grease. Other ways of producing stable, non-bleeding greases have been attempted by either reducing the soap content generally to less than about 5% by weight or by increasing the soap content to a high level. These methods of stabilizing greases against bleeding have also proved to be unsatisfactory because in the case of reducing the soap content to less than 5%, such greases become limited in their use due to the low soap content, while increasing the soap content to a maximum makes the grease too costly and such products generally possess an undesired consistency.

The cause or causes of age-hardening of greases is not understood at present. It is believed to be caused by the soap fibers in storage tending to recrystallize at points of contact to form a more rigid matrix and thus give rise to increased consistency. Such hardening is extremely undesirable for it introduces numerous lubricating difficulties, such as in pumping equipment, and the like.

2

It is an object of this invention to produce greases which are resistant to bleeding and age-hardening. It is a further object of this invention to produce greases by known means, said greases containing additives which prevent age-hardening and bleeding of said greases. Furthermore, it is an object of this invention to produce general all-purpose non-bleeding, non-age-hardening greases containing a minimum amount of soap. Still another object of this invention is to provide a method of making and cooling greases either in a batch or continuous process whereby mechanically stable, non-bleeding products are produced which are resistant to age-hardening.

Now it has been found that the above and other objects of this invention may be attained by adding to a grease composition a minor amount (but sufficient to inhibit oxidation, bleeding and age-hardening) of an oxidized petroleum hydrocarbon rich in aromatics having an aniline point of 75° C. or less, and preferably having an aniline point of 65° C. or less, preferably between 25° and 65° F. Mixtures of said oxidized aromatic-rich petroleum hydrocarbons and/or certain specific fractions thereof, such as nitrogenous and/or sulfurous fractions, can be used also and derivatives thereof. These highly aromatic hydrocarbons may be obtained from various petroleum stocks rich in aromatics by selective solvent treatment, the solvents used in the treatment of a suitable petroleum stock being adapted to segregate the aromatic constituents from the non-aromatic constituents present in the petroleum stock. Suitable solvents may be represented by sulfur dioxide, phenol, furfural, nitrobenzene, cresol, aniline, beta,beta-dichloro-diethyl ether and the like. Petroleum hydrocarbons which are particularly suitable for treatment with the above types of solvents and mixtures thereof are those in the lubricating oil ranges, namely petroleum fractions boiling above about 700 F., such as mineral lubricating oils obtained from crudes rich in aromatics. Particularly preferred are aromatics obtained by the solvent treatment of petroleum distillates having a Saybolt Universal Viscosity of between about 20 and about 200 at 210° F.

Table A gives properties of typical petroleum distillates useful for the extraction of aromatic fractions which are to be subsequently oxidized and used as an additive in accordance with the present invention.

TABLE A

## Properties of petroleum distillate sources

| Sample.....                   | A    | B    | C    | D    | E   | Range of products |
|-------------------------------|------|------|------|------|-----|-------------------|
| Viscosity, SUS at 210.....    | 60   | 39.5 | 50.3 | 70.5 | 158 | 20-200            |
| Aniline point, °F.....        | 64.8 |      |      |      |     |                   |
| Viscosity index.....          | -53  | 90   | 90   | 95   | 92  | -100 to +100      |
| Average molecular weight..... | 364  |      |      |      |     | 225-650           |
| Flash, °F.....                | 370  | 445  | 500  | 570  |     | 350-600           |
| Percent aromatics.....        |      | 15   | 9    | 12   | --- | 2-25              |

Instead of using the entire aromatic component as obtained from a petroleum distillate in the manner described above, the nitrogen or sulfur containing heterocyclic fraction thereof, such as the nitrogenous bases, can also be utilized. The nitrogenous fractions thus obtained consist of mixtures of compounds of carbon, hydrogen and nitrogen, and are probably such compounds as substituted pyridine, quinoline, piperidine, indole, carbazole, pyrazine, cinnoline, naphthyridine, and homologues thereof. Also, the sulfur-

5

taining an Edeleanu extract during its manufacture. Obviously, oxygen or any oxygen-containing fluid may be used in lieu of air. Also, chemical oxidation may be resorted to.

If the aromatic distillates or fractions thereof are oxidized prior to their addition to a grease, they may be oxidized by blowing with an oxidizing gas, such as air, air enriched with oxygen, pure oxygen, hydrogen peroxide, manganese dioxide, permanganates, chlorates, perchlorates, perborates, chromates, chromic acid, etc., preferably under conditions that do not cause the formation of organic peroxides.

Table C presents the properties of several typical oxidized aromatic fractions together with the conditions of oxidation. It will be understood that Table C gives the properties of aromatic fractions which have been oxidized prior to their incorporation in grease compositions. However, when the same aromatic fractions are first incorporated in greases or grease forming components and later subjected to oxidation, substantially the same end products are formed.

TABLE C  
Preparation and properties of oxidized aromatic fractions

| Sample.....                                       | A                                                       | B                                                              | C                                    | Range of products |
|---------------------------------------------------|---------------------------------------------------------|----------------------------------------------------------------|--------------------------------------|-------------------|
| Source.....                                       | Furfural extract of bulk distillate, 200 SUS at 210° F. | SO <sub>2</sub> extract of bulk distillate, 100 SUS at 210° F. | Duo-Solextract of a bulk distillate. | -----             |
| Air blowing conditions:                           |                                                         |                                                                |                                      |                   |
| Time, hours.....                                  | 4.4                                                     | 4.7                                                            | 5.9                                  | 0.5-8             |
| Temp, °F.....                                     | 430                                                     | 430                                                            | 430                                  | 300-500           |
| Oxidation during grease formation, temp., °F..... |                                                         |                                                                |                                      | 175-410           |
| Properties of blown product:                      |                                                         |                                                                |                                      |                   |
| Acid number (mg KOH/g).                           | 0.45                                                    | 0.45                                                           | 0.30                                 | 0.25-5.0          |
| Approx. percent hydrocarbons:                     |                                                         |                                                                |                                      |                   |
| Oxidized.....                                     | 1%                                                      | 1%                                                             | 0.7%                                 | 0.5-25.0          |
| Flash, °F.....                                    | 475                                                     | 470                                                            | 500                                  | 400-600           |
| Softening point, °F.....                          | 121                                                     | 120                                                            | 123                                  | 0-200             |

ous fractions which may be present in the aromatic fractions obtained from petroleum distillates by the Edeleanu process or the like may be used as additives in grease compositions of this invention, such as substituted thiophene, benzothiophene, dibenzothiophene, and homologues thereof.

Table B below gives the properties of suitable aromatic fractions prior to their oxidation.

45

The amount of oxidized products of this invention which can be used as an additive may vary over wide limits and depends upon various factors, such as the lubricant base used to form the grease, the amount and type of soap and other thickening agents used, and the like. Generally, the amount of oxidized product used varies from about 1% to about 20%, and preferably from about 4% to about 10%, of the total composition.

50

The soap used to make greases of this invention (which must contain the oxidized product as described above) may be made by saponification of various fats, fatty acids, derivatives of fats and oils such as fatty acids derived from vegetable, animal, marine and fish oils, and hydrogenated fatty acids thereof, preferably containing from 8 to 40 carbon atoms, synthetic fatty acids produced from hydrocarbons such as oxidizing petroleum products which may be either natural or synthetic, naphthenic acids, rosin acids, tall oil acids, as well as acids of the above type which contain substituent polar groups such as hydroxy, keto, halogen, amino groups and the like. Free glycerine in small amounts up to about 1% may be present in these acid products.

55

Specifically, the natural fats and fatty acid materials derived therefrom which can be used to form soaps include:

I. *Animal*.—Tallow (beef, mutton, goat) etc., lard oil, bone oil, neat's-foot oil, wool fat, horse fat oil, etc.

II. *Vegetable oils*.—Castor oil, cashew nut oil, peanut oil, cocoanut oil, jojoba seed oil, olive oil,

TABLE B

## Properties of aromatic fractions prior to oxidation

| Sample.....               | A   | B    | C    | D   | E     | Range of products |
|---------------------------|-----|------|------|-----|-------|-------------------|
| Visc., SUS at 210° F..... | 106 | 43.7 | 66.8 | 446 | 1,358 | 45-1,500          |
| Iodine No. (Wij's)        | 100 | 96   | 84   | 105 | 113   | 80-150            |
| Aniline point, °F.....    | 32  |      |      |     |       | 25-75             |
| Distillation, 1 mm.:      |     |      |      |     |       |                   |
| IBP, °C.....              | 182 | 135  | 187  | 217 |       | 125-225           |
| 95%, °C.....              | 293 | 239  | 256  | 301 | 346   | 225-400           |

The above aromatic distillates and fractions and/or derivatives thereof may be oxidized by any suitable means either prior to or during their addition to a grease composition. Thus a pre-oxidized Edeleanu extract may be added to a grease composition during the process of making the grease or after the grease has been made, or an Edeleanu extract can be added to a grease composition during some appropriate stage of its manufacture and oxidized therein. This may be accomplished by simply exposing to the air or blowing air through a grease composition con-

60

65

70

75

palm oil; corn oil; cottonseed oil; rapeseed oil; Ravicon oil; sesame oil; soybean oil; linseed oil; etc.

III. *Marine and fish oils*.—Codfish oil, codliver oil, dog fish oil, dolphin oil, herring oil, Menhaden oil, porpoise oil, salmon oil, sardine oil, seal oil, shark oil, whale oil, etc.

IV. Hydrogenated residuum or distillate fractions obtained from any of the oils listed above.

V. Specific fatty acids which can be used to 10 form the soap may include saturated alkyl monocarboxylic acids: Capric, undecylic, lauric, myristic, palmitic, stearic, arachidic, linoceric, montanic, melistic acids, etc.

V(a) *Unsaturated alkyl monocarboxylic acids*.

—Oleic, linoleic, erucic, elupanodonic, linolenic, brassidic, elaidic, elacostearic, stearoleic acids, etc.

V(b) *Hydroxy alkyl carboxylic acids*.—Dimethyl hydroxy caprylic, dimethyl hydroxy capric, ricinoleic, ricinolaidic, 12-hydroxy stearic, 10,11-dihydroxy stearic acid, 4-hydroxy palmitic acid, linusic, sativic, lanoceric, dihydroxy behenic acids, etc. The preferred hydroxy fatty acids are those in which the hydroxy group is at least 12 carbon atoms removed from the carboxyl group.

V(c) *Keto acids*.—Licanic, 12-keto stearic, 13-keto behenic, jojoba oil fatty acids, etc.

VI. *Miscellaneous acids*.—Acids produced by oxidation of hydrocarbons, e. g. paraffin wax, 30 mercapto oleic acid, mercapto stearic acid, amino fatty acids, etc.

Mixtures of fatty materials and derivatives thereof may be used to form soap. Thus, an excellent soap for grease composition may be made from a mixture of hydrogenated fish oil fatty acids and hydrogenated castor oil. When using mixtures of fatty materials in order to form a soap, the fatty materials may vary for example from about 10% of a hydroxy fatty acid and 90% hydrogenated fatty oil and/or its fatty acid derivatives to about 90% of a hydroxy fatty acid and 10% hydrogenated fatty oil product. When using hydroxy fatty acids in a mixture of fatty materials it is preferable to keep the hydroxy fatty acids in the range of between about 50% to 90% by weight. The proportions used are governed in part by the type of mineral oil base used for compounding the greases as well as its intended use.

The soap may be made by saponifying the above type fatty materials, their mixtures, with metal oxide, hydroxides, carbonates, etc., or in the presence of several metal compounds, or organic bases.

A. Metals selected from the Periodic Table, e. g., Group I—lithium, sodium, potassium, rubidium, cesium.

Group II—calcium, strontium, barium, beryllium, magnesium, zinc, cadmium.

Group III—aluminum, gallium, indium.

Group IV—zirconium, tin, lead.

Group V—bismuth.

Group VI—chromium.

Group VII—manganese.

Group VIII—iron, cobalt, nickel.

B. Organic bases such as organic nitrogen bases, e. g., cyclohexylamine, trimethyl cyclohexylamine, ethanolamine, dodecylamine, amyl hexylamine, dicyclohexylamine, triamylamine, quaternary ammonium bases, etc.

Greases prepared from the fatty acid soaps of the alkali or alkaline earth metals, e. g. sodium, lithium, calcium, barium, strontium, and magnesium and their mixtures, as well as the alumini-

num and zinc soap greases, are particularly inhibited against bleeding and age-hardening by addition thereto of the oxidized products of this invention.

5 Instead of making a soap, pre-made soaps can be used to form the grease.

The lubricating oil used for compounding grease of this invention may be of wide viscosity range varying from about 150 Saybolt Universal Viscosity at 100° F. to about 2000 Saybolt Universal Viscosity at 100° F. The viscosity index of the oil can vary from below zero to about 100 and have an average molecular weight ranging from about 250 to 600. It may be highly refined and solvent treated by any known means. A preferred mineral oil is one which has a viscosity between about 300 to 700 SUS at 100° F., a viscosity index of from about 40 to 70 and an average molecular weight of between about 350 and 550.

20 Instead of using straight mineral oil as the base, synthetic oils and lubricants may be substituted in part or wholly for the mineral oil. Among the synthetic lubricants which can be used are: Polymerized olefins, organic esters, e. g. 2-ethylhexyl sebacate, dioctyl phthalate, trioctyl phosphate, polymeric tetrahydrofuran, silicones, etc. Under some conditions of lubrication minor amounts of a fixed oil, such as castor oil, lard oil and the like, may be admixed with the hydrocarbon oil and/or synthetic oil used in making a grease composition of this invention.

25 In accordance with the present invention the oxidized highly aromatic compounds and/or their derivatives can be added to or prepared in the grease at any time during or after the cooking operation. If other additives are to be added they can also be added at any suitable time before, during or after the oxidized highly aromatic 30 additive and/or its derivatives has been added to the grease.

35 Highly desirable greases may be prepared by using formulation within the following range:

|                                                      | General | Preferred |
|------------------------------------------------------|---------|-----------|
|                                                      | range   | range     |
| Soap                                                 | Percent | Percent   |
| Oxidized products of this invention                  | 5-25    | 7-14      |
| Polyalkylene glycol and/or its derivatives           | 1-20    | 4-10      |
| Hydrocarbon oil (viscosity 150-2,000 SUS at 100° F.) | 0-1     | 0.01-0.1  |
|                                                      | 54-94   | 75.9-88.9 |

40 Grease compositions of this invention may be made in the following manner using as an example the following components:

|                                                                                      | Components | Lb./100 lb. grease |
|--------------------------------------------------------------------------------------|------------|--------------------|
| Hydrogenated fish oil acids                                                          |            | 7.0                |
| Hydrogenated castor oil                                                              |            | 1.0                |
| 60 Polyethylene glycol having an average molecular weight of 600                     |            | .045               |
| Sodium hydroxide (dissolved in 2 lbs. water)                                         |            | 1.12               |
| Oxidized Edelenmu extract (derived from 60 SUS at 210° F. petroleum bulk distillate) |            | 5.0                |
| Mineral lubricating oil 600 SUS at 100° F.                                           |            | 86.3               |

65 The acids and glycerides are melted with about twice their weight of oil at about 80° C. and caustic solution is added. The precipitated soap is vigorously stirred to form a slurry and heated to drive off the water. During the heating and stirring, a modicum of polymeric silicone, e. g., dimethyl silicone polymer, can be added to inhibit foaming. Heating is continued with efficient stirring until a temperature of about 340° F. is reached. At this point hot oil (250° F.) con-

taining oxidized Edeleanu extract is slowly blended in with the oil-soap slurry and the entire mixture is heated so as to maintain the soap-oil mixture in a gelatinous state. If the Edeleanu extract is not oxidized prior to its addition to the soap-like mixture, the entire mixture should be exposed to the atmosphere so that the Edeleanu extract can be oxidized while the grease is being formed. The polyethylene glycol is usually added during the addition of the hot oil to the soap-oil mixture. The final mixture is heated to about 360° F. but below about 410° F. and then transferred to a suitable container for heat conditioning.

To illustrate the profound effect oxidized Edeleanu extract and non-oxidized Edeleanu extract has on the age-hardening of a grease the following experiment was made, the results of which are noted in the table below and plotted in the figure. One sample of a sodium soap grease, as described above, was prepared in an open kettle so as to allow the Edeleanu extract to become oxidized, and the other sample of a sodium soap grease containing the same materials was prepared in an atmosphere of nitrogen gas so as to prevent oxidation of the Edeleanu extract. As the figure shows, the two greases were tested periodically during storage after their preparation. According to the figure, after an initial 2 weeks period of equal hardening, the rate of hardening of the grease containing oxidized extract (see Curve A) suddenly retarded, while the grease containing unaltered extract (see Curve B) continued to harden at its original high rate.

Age hardening of soda-base grease

| Composition                                                                                                 | ASTM penetration | Penetration change after 8 weeks |
|-------------------------------------------------------------------------------------------------------------|------------------|----------------------------------|
| Soda base grease containing 5% oxidized Edeleanu extract derived from 60 SUS at 210° F. bulk distillate     | 352              | 19                               |
| Soda base grease containing 5% non-oxidized Edeleanu extract derived from 60 SUS at 210° F. bulk distillate | 295              | 40                               |

Grease compositions of this invention may be prepared by any other suitable means known in the art and cooled either slowly or rapidly depending upon the type of soap used to make the grease. Thus, if soda soap or alkaline earth greases are made they may be cooled slowly in the kettle, whereas if lithium or aluminum soap greases of this invention are made it is preferred that they be cooled uniformly and rapidly either in tubes of small diameter or in thin layers by feeding the hot grease onto a steel belt and subjecting the grease to a current of air or other cooling medium, so as to cool the grease in a uniform fashion free from shearing stresses.

Additional stabilizing agents may be incorporated in these greases. A particularly desirable type of stabilizing agent which can be used with grease compositions of this invention includes the alkylene glycol and/or alkylene thio glycol polymers as well as their mono-esters and ether polymeric derivatives. The alkylene glycol polymeric materials can be represented by the following general structural formula:



wherein  $m$  and  $n$  and  $a$  are integers. Preferably the polymeric alkylene glycols as represented by the above general formula should be such that

75

the factor  $a$  times the number of carbon atoms within the brackets should be at least 6 and more.

The polymeric alkylene glycols can be made by polymerizing in the presence of a catalyst such as iodine, hydriodic acid and the like, ethylene, propylene, isobutylene, n-butylene oxides and/or their mixtures. Such polymers can also be produced by reacting a monohydric alcohol with an alkylene oxide. Thus, a suitable product can be made by reacting n-butanol with propylene oxide at between about 212 to 230° F. under pressure and in the presence of an alkali catalyst.

The polymerized higher polyalkylene glycols having between 2 and 6 carbon atoms in the alkylene group are most effective as additives of this invention and those containing the ethylene and propylene groups are preferred. The average molecular weight of the polyalkylene glycols may be from about 200 to about 7000 and the preferred molecular weight being from about 1000 to 6000.

It is desired to point out that the higher polyalkylene glycols are composed of mixtures of several polymers, for example, a polyethylene glycol having an average molecular weight of 400 consists of various glycols varying from a minor amount of monoethylene glycol and increasing up to the pentadecaethylene glycol. Therefore, it is the average molecular weight which is specified and where in the present specification polyalkylene glycols or polyethylene glycols are referred to, they define the higher glycols having an average molecular weight in excess of 200 and preferably in excess of 400, those with an average molecular weight of between about 1000 to 1500 being very effective in carrying out the present invention.

In lieu of the polyalkylene glycols, the ester and ether derivatives can be used. The esters can be made from a variety of acids having between 2 to about 22 carbon atoms and preferably between about 10 to 18 carbon atoms. Acids which may be used are the aliphatic, aromatic, cyclic, sulfonic acids and the like. Fatty acids and especially the higher fatty acids are preferred and include such acids as lauric, myristic, palmitic, stearic, arachidic, behenic, oleic, ricinoleic, hydroxy stearic, phenylacetic, phenyl stearic acids and the like. However, such acids as naphthenic acid, oil-soluble petroleum sulfonic acids, tall oil fatty acids, aromatic acids, e. g. salicylic and phthalic acids and the like may be used to form the esters. Specific examples of esters of this type are the polyethylene glycol monostearate, polyethylene glycol monooleate and the like.

Ether derivatives of polyalkylene glycols may be made by any conventional method and the aromatic ethers of polyalkylene glycols having the general formula:



wherein  $Ar$  is an aromatic radical having attached thereto at least one alkyl radical denoted by  $R'$  having from 1 to about 8 carbon atoms and wherein  $Y$  is a fatty acid derivative,  $n$ ,  $m$  and  $a$  are integers as in I and  $q$  is a number selected from the group consisting of zero or 1.

Thio alkylene glycol polymers can be represented by the general formula:



wherein  $m$ ,  $n$  and  $r$  are integers and  $R$  is an organic radical, preferably a hydrocarbon. These

materials can be prepared by reacting an alkylene glycol or an alkylene oxide with an alkylene sulfide, e. g. ethylene, propylene, amylene sulfides, thio glycol or mercaptans.

The average molecular weight of the poly-alkylene glycol derivatives can be below 400 and up to about 7000, the derivatives having an average molecular weight of between 700 to about 7000 are preferred.

The amount of polyalkylene glycol derivatives thereof or other anti-bleeding agent which can be used depends upon the soap concentration and in part upon the type of oil base used. However, it has been found that it is not necessary to use more than 1% by weight of these additives although larger amounts can be used if desired. Generally effective results are obtained with concentrations ranging from 0.01 to about 0.5% and preferably when kept within the range of between about 0.05 to about 0.25% by weight.

To further illustrate the present invention the following example is presented.

In a suitable open grease-making kettle approximately 3.7% of hydrogenated fish oil fatty acids and 3.7% of hydrogenated castor oil fatty acids, 1.0% lithium hydrate solution and about 10% of a 100 SUS at 100° F. paraffin oil can be admixed and heated while stirring to a temperature of between about 380° F. and about 400° F. To this mixture about 35 to 40% of 100 SUS at 100° F. paraffin oil, 30% 2000 SUS at 100° F. Coastal Pale Oil and about 5% to 15% of oxidized Edeleanu extract derived from a 60 SUS 210° F. bulk distillate is added very slowly and the temperature of the mixture maintained at between about 380 to 385° F. When a homogeneous mass is formed about 0.01% polyethylene glycol is added to the grease. The hot fluid mass can be poured into flat pans to a depth of less than 1 inch and exposed to a current of cooling air so that the grease cools down to around about 150° F. in less than 30 minutes. The cooled grease forms an improved non-bleeding lithium soap grease upon milling. The oxidized Edeleanu extract to be used in this test may be obtained by air blowing the extract at a temperature of about 425° F. for about 4 hours.

The process of making the above grease was repeated except that the oxidized Edeleanu extract was omitted.

The above lithium soap greases were tested for bleeding in accordance with the Army-Navy Aeronautical specification for greases AN-G-25 of April 10, 1946. The sample containing oxidized Edeleanu extract showed no tendency toward bleeding while the sample from which oxidized Edeleanu extract was omitted showed marked tendency towards bleeding.

During the cooking of the above lithium grease, there may be introduced small amounts of soaps or salts, generally in amounts of less than 2% for additional benefits. For example, there may be incorporated into a lithium soap grease, as described above, a minor amount of aluminum or sodium soap or alkali and alkaline earth naphthenates, acetates, etc.

Minor amounts of oxidation inhibitors can be added to grease compositions of this invention such as N-butyl paraphenylenediamine. Also effective as oxidation inhibitors are alpha or beta naphthylamine, phenyl-alpha or beta naphthylamine, alpha-alpha, beta-beta, or alpha-beta dinaphthylamine, diphenylamine, tetramethyl diamino diphenylmethane, petroleum alkyl phenols, and 2,4-ditertiary butyl 6-methyl phenol.

Corrosion inhibitors which are particularly

applicable with compositions of this invention are N-primary amines containing at least 6 and more than 18 carbon atoms in the molecule such as hexylamine, octylamine, decylamine, dodecylamine, octadecylamine, heterocyclic nitrogen containing organic compounds such as alkyl substituted oxazolines and oxazole salts of fatty acids.

Extreme pressure agents can be added to such grease and the preferred agents comprise esters of phosphorus acids such as triaryl, alkylhydroxy, aryl, or aralkyl phosphates, thio-phosphates or phosphites, etc., neutral aromatic sulfur compounds such as diaryl sulfides and polysulfides, e. g. di-henyl sulfide, diresol sulfide, cibenzyl sulfide, methyl butyl diphenol sulfide, etc., diphenyl selenide and diselenide, diresol selenide and polyselenide, etc., sulfurized fatty oils or esters of fatty acids and monohydric alcohols, e. g. sperm oil, jojoba oil, etc., in which the sulfur is tightly bound; sulfurized long-chain olefins obtained by dehydrogenation or cracking of wax; sulfurized phosphorus acids with hydroxy fatty acids, chlorinated hydrocarbons such as chlorinated paraffins, aromatic hydrocarbons, terpenes, mineral lubricating oils, etc.; or chlorinated esters of fatty acids containing the chlorine in positions other than the alpha position.

Additional ingredients which can be added are anti-wear agents such as oil-soluble urea or thio-urea derivatives, e. g. urethanes, allophanates, carbazides, carbazones, etc.; or rubber, polyisobutylene, polyvinyl esters, etc.; VI improvers such as polyisobutylene having a molecular weight above about 800, volatilized paraffin wax, unsaturated polymerized esters of fatty acids and monohydric alcohols, etc.; oiliness agents such as stearic and oleic acids and pour point depressors such as chlorinated naphthalene to further lower the pour point of the lubricant.

The amount of the above additives can be added to grease compositions of this invention in around about 0.01% to less than 10% by weight and preferably 0.1 to 5.0% by weight.

Greases of this invention are applicable for general automotive uses, and are excellent aircraft greases, industrial greases and the like.

This case is a continuation-in-part of the co-pending application, Serial No. 40,727 filed July 26, 1948, now abandoned.

I claim as my invention:

1. A lubricating grease comprising a major amount of a mineral lubricating oil having a viscosity index of from 40 to 70, about 5% to 25% of a soda soap of a higher fatty acid, from 0.01% to 0.1% of polyethylene glycol having an average molecular weight of 600, and from 4% to 10% of an oxidized petroleum aromatic extract fraction obtained by solvent treatment of a petroleum distillate having a viscosity of 60 SUS at 210° F., said aromatic extract fraction having an aniline point between 25 and 75° C., and said oxidized petroleum fraction having been formed by exposure of the fraction and the grease forming components to air during grease forming operations at a temperature between about 175° F. and about 410° F.

2. A lubricating grease comprising a major amount of a mineral lubricating oil having a viscosity index of from 40 to 70, about 5% to 25% of a lithium soap of a higher fatty acid, from 0.01% to 0.1% of polyethylene glycol having an average molecular weight of 600, and from 4% to 10% of an oxidized petroleum aromatic extract

fraction obtained by solvent treatment of a petroleum distillate having a viscosity of 60 SUS at 210° F., said aromatic extract fraction having an aniline point between 25 and 75° C. and said oxidized petroleum fraction having been formed by exposure of the fraction and the grease forming components to air during grease forming operations at a temperature between about 175° F. and about 410° F.

3. A lubricating grease comprising a major amount of a mineral lubricating oil having a viscosity index of from 40 to 70, about 5% to 25% of a lithium soap of a mixture of hydrogenated fish oil acids and hydrogenated castor oil, from 0.01% to 0.1% of polyethylene glycol having an average molecular weight of 600, and from 4% to 10% of an oxidized petroleum aromatic extract fraction obtained by solvent treatment of a petroleum distillate having a viscosity of 60 SUS at 210° F., said aromatic extract fraction having an aniline point between 25 and 75° F., and said oxidized petroleum fraction having been formed by exposure of the fraction and the grease forming components to air during grease forming operations at a temperature between about 175° F. and about 410° F.

4. A lubricating grease comprising a major amount of a mineral oil having a viscosity index greater than 40, a minor amount of a soap to thicken the oil, and from about 1% to about 20% by weight of an oxidized petroleum aromatic extract fraction obtained by solvent treatment of a petroleum distillate having a viscosity of 60 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F.

5. A lubricating grease comprising a major amount of a mineral oil having a viscosity index greater than 40, a minor amount of a soda soap to thicken the oil and a minor amount of from about 1% to about 20% sufficient to prevent age-hardening of the grease of an oxidized petroleum aromatic extract fraction obtained by solvent treatment of a petroleum distillate having a viscosity of 60 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F.

6. A lubricating grease comprising a major amount of a mineral oil having a viscosity index greater than 40, a minor amount of a lithium soap to thicken the oil and a minor amount of from about 1% to about 20% sufficient to prevent age-hardening of the grease of an oxidized petroleum aromatic extract fraction obtained by solvent treatment of a petroleum distillate having a viscosity of 60 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F.

7. A lubricating grease comprising a major amount of a mineral oil having a viscosity index greater than 40, a minor amount of an aluminum soap to thicken the oil and a minor amount of from about 1% to about 20% sufficient to prevent age-hardening of the grease of an oxidized

petroleum aromatic extract fraction obtained by solvent treatment of a petroleum distillate having a viscosity of 60 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F.

10 8. A lubricating grease comprising a major amount of a mineral oil having a viscosity index greater than 40, a minor amount of a soap to thicken the oil and a minor amount of from about 1% to about 20% sufficient to prevent age-hardening of the grease of an oxidized petroleum aromatic extract fraction obtained by solvent treatment of a petroleum distillate having a viscosity of 60 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F., and a minor amount, but less than 1% of a polyalkylene glycol having an average molecular weight of between about 400 to about 7000.

9. A lubricating grease comprising a major amount of a mineral oil having a viscosity index greater than 40, a minor amount of a soda soap to thicken the oil and a minor amount of from about 1% to about 20% sufficient to prevent age-hardening of the grease of an oxidized petroleum aromatic extract fraction obtained by solvent treatment of a petroleum distillate having a viscosity of 60 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F., and a minor amount, but less than about 1% of a polyalkylene glycol having an average molecular weight of between about 400 to about 7000.

40 10. A lubricating grease comprising a major amount of a mineral oil having a viscosity index greater than 40, a minor amount of a lithium soap to thicken the oil and a minor amount of from about 1% to about 20% sufficient to prevent age-hardening of the grease of an oxidized petroleum aromatic extract fraction obtained by solvent treatment of a petroleum distillate having a viscosity of 60 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F., and a minor amount, but less than about 1% of a polyalkylene glycol having an average molecular weight of between about 400 to about 7000.

11. A lubricating grease comprising a major amount of a mineral oil having a viscosity index greater than 40, a minor amount of an aluminum soap to thicken the oil and a minor amount of from about 1% to about 20% sufficient to prevent age-hardening of the grease of an oxidized petroleum aromatic extract fraction obtained by solvent treatment of a petroleum distillate having a viscosity of 60 SUS at 210° F., said oxidized petroleum aromatic extract fraction having been formed by exposure of the fraction and the grease forming components to air during grease forming operations at a temperature between

about 175° F. and about 410° F., and a minor amount, but less than about 1% of a polyalkylene glycol having an average molecular weight of between about 400 to about 7000.

12. A lubricating grease comprising a major amount of a lubricating oil having a viscosity index greater than about 40, and a minor amount of a soap and from about 1% to about 20% by weight of the grease of an oxidized petroleum aromatic extract fraction obtained by solvent treatment of a petroleum distillate having a viscosity of from about 20 to about 200 SUS at 210° F., said aromatic extract fraction having an aniline point between about 25 and about 75° C., and said oxidized fraction having been formed by exposure of said fraction to an oxygen containing gas at a temperature between about 175 and about 500° F.

13. A lubricating grease comprising a major amount of a mineral oil having a viscosity index greater than about 40, and a minor amount of a soap and from about 1% to about 20% by weight of the grease of an oxidized petroleum aromatic extract fraction obtained by solvent treatment of a petroleum distillate having a viscosity of from about 20 to about 200 SUS at 210° F., said aromatic extract fraction having an aniline point between about 25 and about 75° C., and said oxidized fraction having been formed by exposure of said fraction to an oxygen containing gas at a temperature between about 300 and about 500° F. prior to incorporation in the grease.

14. A lubricating grease comprising a major amount of a mineral oil having a viscosity index greater than about 40, and a minor amount of a soap and from about 1% to about 20% by weight of the grease of an oxidized petroleum aromatic extract fraction obtained by solvent treatment of a petroleum distillate having a viscosity of from about 20 to about 200 SUS at 210° F., said aromatic extract fraction having an aniline point between about 25 and about 75° C., and said oxidized fraction having been formed by exposure of said fraction to an oxygen containing gas at a temperature between about 300 and about 500° F. prior to incorporation in the grease for a period between about 0.5 and about 8 hours.

15. A lubricating grease comprising a major amount of a mineral lubricating oil having a viscosity index of at least 40, a minor amount of a soap and from about 1% to about 20% by weight of the grease of an oxidized petroleum aromatic extract fraction obtained by solvent treatment of a petroleum distillate having a viscosity of from about 20 to about 200 SUS at 210° F., said aromatic extract fraction having an aniline point between about 25 and about 75° C., and said oxidized fraction having an acid number between about 0.25 and 5.0 mg. KOH per gram and having between about 0.5 and about 25% of its molecules in an oxidized state.

16. A lubricating grease comprising a major amount of a mineral oil having a viscosity index greater than about 40, less than about 1% of a polyalkylene glycol having an average molecular weight between about 400 and about 7,000, and a minor amount of a soap and from about 1% to about 20% by weight of the grease of an oxidized petroleum aromatic extract fraction obtained by solvent treatment of a petroleum distillate having a viscosity of from about 20 to about 200 SUS at 210° F., said aromatic extract fraction having an aniline point between about 25 and about 75° C., and said oxidized fraction having been formed by exposure of said fraction to an oxygen containing gas at a temperature between about 300 and 75

about 500° F. prior to incorporation in the grease for a period between about 0.5 and about 8 hours.

17. A lubricating grease comprising a major amount of a lubricating oil having a viscosity index greater than about 40, and a minor amount of a metallic soap of a higher aliphatic monocarboxylic acid and from about 1% to about 20% by weight of the grease of an oxidized petroleum aromatic extract fraction obtained by solvent treatment of a petroleum distillate having a viscosity of from about 20 to about 200 SUS at 210° F., said aromatic extract fraction having an aniline point between about 25 and about 75° C., and said oxidized fraction having been formed by exposure of said fraction to an oxygen containing gas at a temperature between about 175 and about 500° F.

18. A lubricating grease comprising a major amount of a lubricating oil having a viscosity index greater than about 40, and a minor amount of an alkali metal soap of a higher fatty acid and from about 1% to about 20% by weight of the grease of an oxidized petroleum aromatic extract fraction obtained by solvent treatment of a petroleum distillate having a viscosity of from about 20 to about 200 SUS at 210° F., said aromatic extract fraction having an aniline point between about 25 and about 75° C., and said oxidized fraction having been formed by exposure of said fraction to an oxygen containing gas at a temperature between about 175 and about 500° F.

19. A lubricating grease comprising a major amount of a mineral oil having a viscosity index greater than 40, a minor amount of a soap to thicken the oil, and from about 1% to about 20% by weight of an oxidized petroleum aromatic extract fraction obtained by solvent treatment of a petroleum distillate having a viscosity of from about 20 to about 200 SUS at 210° F., said aromatic extract fraction having an aniline point between 25 and 75° C., said oxidized solvent fraction having been formed by exposure of the fraction and the grease forming components to air during grease forming operations at a temperature between about 175° F. and about 410° F.

20. The process which comprises forming a mixture of a lubricating oil having a viscosity index greater than 40, a minor amount of a soap to thicken the oil and from about 1% to about 20% by weight of a petroleum aromatic extract fraction obtained by solvent treatment of a petroleum distillate having a viscosity of from about 20 to about 200 SUS at 210° F., said aromatic extract fraction having an aniline point between 25 and 75° C., and exposing the mixture to air during grease forming operations at a temperature between about 175° F. and about 410° F. whereby said aromatic extract fraction is oxidized.

60

ROBERT J. MOORE.

## REFERENCES CITED

The following references are of record in the file of this patent:

## UNITED STATES PATENTS

| Number    | Name           | Date          |
|-----------|----------------|---------------|
| 1,971,750 | Kaufman        | Aug. 28, 1934 |
| 2,057,473 | Burch          | Oct. 13, 1936 |
| 2,128,574 | Van Peski      | Aug. 30, 1938 |
| 2,245,772 | Gothard et al. | June 17, 1941 |
| 2,326,596 | Zimmer et al.  | Aug. 10, 1943 |
| 2,343,125 | Larsen         | Feb. 29, 1944 |
| 2,403,104 | Lien           | July 2, 1946  |
| 2,445,935 | Bondi          | July 27, 1948 |